

## UNITED STATES PATENT OFFICE

2,153,390

## LEADING-IN WIRE FOR ELECTRIC DEVICES

Marcello Pirani, Berlin-Wilmersdorf, and Hans Wolff, Zeuthen, Germany, assignors to General Electric Company, a corporation of New York

No Drawing. Application December 14, 1933, Serial No. 702,425. In Germany January 6, 1933

3 Claims. (Cl. 49—92)

Our invention relates to leading-in wires for electric devices comprising a glass bulb or enclosure and more particularly to a new composition for leading-in wires sealed in a bulb of boron-silicate glass which has a higher melting point than the usual lead and calcium glasses.

5 Our new leading-in wire is particularly adaptable for electric discharge tubes comprising a bulb of boron-silicate glass containing less than 10 50 per cent of silicic acid and more than 30 per cent of boric acid with a small amount of alkali. The bulbs of such tubes attain a temperature of several hundred degrees centigrade during operation and contain a filling of a vapor of substances such as sodium, cadmium, magnesium, 15 or thallium.

An object of our invention therefore is to provide a leading-in wire which will form a reliable seal with a hard glass such as boron-silicate glass.

20 According to our invention the new leading-in wire consists of an alloy of tungsten and nickel to which is preferably added a small amount of cobalt. The proportions are preferably 70-85 per cent of tungsten and 15-30 per cent of nickel. Preferably a small part of the nickel, up to 5 per 25 cent of the total quantity of alloy, is replaced by cobalt. This alloy can be readily drawn into wire. The sealing in the glass is improved by the addition of the cobalt while the drawing qualities are not noticeably impaired by it when con-

fined to amounts under five per cent of the total alloy.

The following suitable compositions may be used for the new leading-in wire alloy:

|              | Parts by weight | 5  |
|--------------|-----------------|----|
| (1) Tungsten | 84              |    |
| Nickel       | 12              |    |
| Cobalt       | 4               | 10 |
| (2) Tungsten | 74              |    |
| Nickel       | 22              |    |
| Cobalt       | 4               |    |

What we claim as new and desire to secure by Letters Patent of the United States is:

1. As a new article of manufacture, a leading-in wire consisting of an alloy of tungsten and nickel, said alloy having a coefficient and expansion adapting it to be sealed to hard glass.

2. As a new article of manufacture, a leading-in wire consisting of an alloy of seventy to eighty-five per cent of tungsten and fifteen to thirty per cent of nickel.

3. As a new article of manufacture, a boron-silicate glass article having sealed therein a leading-in wire consisting of an alloy of tungsten and nickel.

MARCELLO PIRANI.  
HANS WOLFF.

20

25

30

CERTIFICATE OF CORRECTION.

Patent No. 2,153,390.

April 4, 1939.

MARCELLO PIRANI, ET AL.

It is hereby certified that error appears in the printed specification of the above numbered patent requiring correction as follows: Second column, line 18, claim 1, for "and" read of; and that the said Letters Patent should be read with this correction therein that the same may conform to the record of the case in the Patent Office.

Signed and sealed this 23rd day of May, A.D. 1939.

(Seal)

Henry Van Arsdale  
Acting Commissioner of Patents.